

1

3,130,125

## PREPARATION OF MEDICATED BENZYL DEXTRAN GRADUAL RELEASE THERAPEUTIC PRODUCTS CONTAINING UP TO FIVE PERCENT BENZYL ALCOHOL

Herman Heckel, Oxford, and Robert T. Jefferson, West Carrollton, Ohio, assignors to The Central Pharmacal Company, Seymour, Ind., a corporation of Indiana  
No Drawing. Filed Sept. 14, 1962, Ser. No. 223,839

2 Claims. (Cl. 167—82)

This invention relates to delayed release medicaments, and more particularly to delayed release medicaments prepared with benzyl dextran.

For numerous purposes it is necessary to administer medicaments over extended periods of time in order to accomplish the desired result. In most cases it is necessary to administer the medicament at stated intervals in order to maintain a useful concentration of the medicament in the body without at the same time having present toxic amounts. It is well known that almost any medicament will produce harmful instead of beneficial results when excessive quantities are introduced into the blood stream of the body, and that too small quantities produce little, if any, beneficial effect, and may even prove harmful in establishing immunity against the medicament. It is accordingly necessary to exercise extreme care in the administration of all medicaments, and in particular those of a high degree of toxicity.

The necessity of maintaining a regulated level of a medicament in the blood stream has in the past made it essential to administer regulated amounts of the medicament at fairly frequent regulated intervals, the amounts and time intervals being dependent upon the particular medicament. In cases where the medicament has a high degree of toxicity or where the rate of excretion from the body is high it has been necessary to administer the drug at quite frequent intervals with resultant inconvenience and cost to the patient, as well as to the physician or nurse.

It is an object of this invention to provide a practical economical means of administering medicaments in a manner so that the required levels of the medicament can be maintained in the body without harm to the patient and without the necessity for frequent dosages of the medicament. This is accomplished by administering the medicament in combination with benzyl dextran, and particularly benzyl dextran of the character described below. By suitably regulating the composition as hereinafter described it is possible to regulate the rate of release of the medicament as desired so that much less frequent dosages are required in order to maintain a particular desired effective concentration of the medicament in the body of the patient being treated. Large dosages of the benzyl dextran-medicament composition are administered in extended periods and by regulating the amount of the medicament or the type of the benzyl dextran used, or both, the medicament will be released in the body to give the particular desired concentration over a particular desired period of time.

The term "dextran" is applied to a class of polymers of glucose having chain-like structures and usually of very high molecular weight, produced by fermentation. The structure of dextran varies somewhat depending upon its method of production. For use in preparing benzyl dextran suitable for delayed release medicament compositions dextran having a ratio of repeating alpha-1,6 to alpha non-1,6 glycosidic links from 2:1 to 32:1 has been found to be particularly suitable. The dextran used to produce synthetic blood-volume expanders falls within this range and has a ratio of repeating alpha-1,6 to alpha non-1,6 glycosidic links of 19:1.

2

The molecular weight of the dextran used in making benzyl dextran for delayed release medicaments should fall preferably within the range of three million to sixty million, determined by light scattering, which is the average molecular weight range for most of the dextrans obtained by normal fermentations. In general, the rate of release of the medicament from the benzyl dextran-medicament composition is increased as the molecular weight is reduced. Where it is desired to speed up the rate of release this can be accomplished by hydrolysis of the native dextran controlled so as to give dextran of any particular molecular weight range.

The degree of substitution of the benzyl in the benzyl dextran also has an important bearing on the rate of release of the medicament from the benzyl dextran-medicament compositions. In general, the rate of release is decreased as the degree of substitution is raised and increased as the degree of substitution is decreased. For most uses, a degree of substitution ranging from 0.8 to 1.0 has been found to be most desirable, a D.S. below 0.8 giving too rapid release for most practical purposes, and above 1.0 not giving fast enough release. For some purposes, however, benzyl dextran having a D.S. of benzyl outside of this range is useful.

25 A benzyl dextran, designed to give gradual release of medicament in the body over a period of eight to sixteen hours, should have a molecular weight ranging from three million to sixty million, a ratio of repeating alpha-1,6 to alpha non-1,6 glycosidic links of 2:1 to 32:1, and preferably 19:1, and in which 26—32% of the replacable hydrogens on the hydroxyl groups have been replaced by benzyl groups (i.e., a D.S. of 0.8—1.0).

The benzyl dextran used in the benzyl dextran-medicament composition can be produced in various ways but 35 preferably by reacting a benzyl halide (Cl, Br, or I) with native dextran in the presence of a strong base (NaOH, KOH) in an aqueous system. Benzyl chloride is the preferred benzyl compound and sodium hydroxide the preferred base. To produce a benzyl dextran having a benzyl D.S. of 0.8—1.0 these reactants are used in the ratio of 4—8 moles of NaOH, 3—5 moles of benzyl chloride, and 75—100 moles of water, per mole of dextran.

The dextran is first dissolved in the water, one-half of the sodium hydroxide added, as a 40% aqueous solution, and the resulting solution heated to 90° C. with constant stirring. At this temperature one-third of the benzyl chloride is slowly added and the resulting mixture heated under reflux at 95—100° C. until the odor of benzyl chloride is no longer detected. During this period 50 the partially substituted benzyl dextran separates as an insoluble soft gum. Water is added to the reaction before any liquid is removed. This operation reduces the concentration of by-products produced in this step of the operation.

55 The second half of the sodium hydroxide in 40% aqueous solution is then added to the soft gum remaining in the reaction vessel and the mixture heated to 90° C. A second one-third portion of the benzyl chloride is next added and the mixture heated under reflux at 95—100° C. until the odor of benzyl chloride is no longer detected. The remaining one-third of benzyl chloride is then added and refluxing continued until the odor of benzyl chloride is no longer detected.

60 The refluxing periods will vary directly with the quantities of reaction products. A reaction mixture containing two moles of dextran will normally require refluxing for about thirty minutes, while one containing 10 moles of dextran will usually require refluxing for approximately one hour to complete the reaction.

65 The benzyl dextran is then recovered and purified by any convenient method, as for example, by washing with

water followed by steam distillation. A preferred method consists of washing with water, solution in an isopropanol-miscible solvent (i.e. monoethyl ether of ethylene glycol), precipitation with isopropanol and drying. The benzyl dextran obtained by the latter method is a substantially white free-flowing amorphous powder having a benzyl D.S. ranging from 0.8 to 1.0 and molecular weight ranging from three million to sixty million, and other impurities and ready for use in preparing delayed release benzyl dextran-medicament compositions. Benzyl dextran prepared and recovered as above described will usually contain not in excess of 1% impurities, and it is such a grade of benzyl dextran that is purposely used in order to reduce to a minimum the toxic ingredients of the benzyl dextran. Benzyl dextran obtained by the first mentioned and other processes frequently is mixed with substantial amounts of benzyl alcohol and other impurities such as benzyl ethers and hence may require further purification, depending upon the character and amount of impurities present. The requirement for and character of additional purification is to a large extent dependent upon the requirements of the United States Food and Drug Administration. For example, the presence of as much as 20% of benzyl impurities (benzyl alcohol and benzyl ether) does not significantly alter the rate of release of a medicament from a benzyl dextran-medicament composition in which the benzyl dextran having a benzyl D.S. of 0.8-1.0, although the maximum amount of these impurities allowed, from a toxicity standpoint, is considered to be about 1%. When, however, the benzyl D.S. is increased above 1.0 the softening temperature of the benzyl dextran is lowered and the presence of 5% or more of benzyl alcohol still further reduces the softening temperature with the result that the benzyl dextran granules flow into a plastic mass at 37° C., and thereby reduce the total surface area to such an extent that the medicament is not readily released from the benzyl dextran-medicament composition.

The mechanism of the combination of the benzyl dextran and medicament is not definitely known. It is believed, however, that the medicament is held in suspension within the tightly coiled molecules of the benzyl dextran without substantial loss through decomposition, vaporization or sublimation during the processing and subsequent storage can be used with the benzyl dextran and administered as a delayed release medicament, the only limitation being that the medicament selected be such that it can be homogeneously suspended in the benzyl dextran and entrapped within its coiled molecules. Analgesics and antiarthritics such as acetophenetidin with aspirin and caffeine and meperidine; antiacids and antidiarrheatics such as magnesium trisilicate; antibiotics such as penicillin, tetracycline, chloramphenicol, erythromycin; anticholinergics such as atropine-phenobarbital; antihistaminics such as chloropropenpyridamine, promethazine; cardiotonics such as pentaerythritol tetranitrate; diuretics such as acetazolamide; psychopharmacological drugs such as chlorpromazine, dextroamphetamine, meprobamate; steroid hormones such as estrogens, hydrocortisone; vasoconstrictors such as phenylephrine; vitamin preparations such as B<sub>12</sub> etc. represents examples of medicaments which can be used with the benzyl dextran in the formulating of delayed release medicaments.

The amount of medicament combined with the benzyl dextran depends to a considerable degree on the desired dosage of the medicament and the influence of the concentration of the medicament on its rate of release from the combination. In the case of dextroamphetamine 5 to 15% of the medicament in the combination has been found satisfactory. Larger amounts may, of course, be used unless the character of the medicament is such that the amount released at any time might be hazardous to the patient. In such cases, however, the benzyl D.S. may be increased so as to slow up the rate of release. This illustrates one of the principal advantages of the use of

benzyl dextran in delayed release medicaments, namely, that the benzyl dextran can be tailor-made to fit the particular medicament and the particular type of treatment required for best results. In other words, by selecting the particular medicament, the concentrations thereof used, and the particular benzyl D.S. a delayed release medicament can be prepared to fit any usual requirement.

The medicament can be incorporated with the benzyl dextran in any suitable manner which will assure homogeneity and entrapment within the benzyl dextran molecules. One convenient method of doing this has been by preparing a fluid paste of the benzyl dextran in methanol using the minimum quantity of methanol—one to three parts of methanol by weight to one part of benzyl dextran. The medicament is then incorporated with the fluidized benzyl dextran in the desired quantity and thoroughly blended by stirring and heating up to 60° C. If the medicament is solid it is generally necessary to incorporate it in solution or suspension form in order to assure thorough mixing. A preferred method is to introduce the medicament in aqueous or methanolic solution or solution in other volatile solvent from which the medicament is not readily precipitated by methanol. The fluid mass, after thorough mixing and incorporation of the medicament, is dried in vacuo at 60° C., or other temperature at which the solvents are readily removed without undesirably affecting either the benzyl dextran or medicament. After drying the mixture is crushed, preferably to pass a #10 mesh screen and retained on a #20 mesh screen. The product can then be administered in the desired dosages in either capsules or in tablet form.

The delayed release characteristics of the benzyl dextran with the medicament are then determined by extracting the medicament with simulated gastro-intestinal fluids under a standard set of conditions. The percent of the total medicament extracted during a series of specific periods of time is plotted on graft paper and the curve compared to specifications. These determinations are carried out as follows:

One thousand milligrams of the benzyl dextran medicament in granular form, prepared as above described, are dispersed in 80 ml. of simulated gastric fluid, pH 1.5 (U.S.P.) in a 250 ml. Erlenmeyer flask, which is then placed on a reciprocating shaker at 37° C. for fifty-five minutes. The residual medicament from this extraction is then dispersed in simulated intestinal fluid, pH 7.5 (U.S.P.) and extracted as described above for the periods of time indicated in the schedule below. The extracts are then assayed for the medicament by any suitable means. The table below shows results obtained as above described for a benzyl dextran-dextro-amphetamine hydrochloride composition containing 5-15% of the medicament, the benzyl dextran having a benzyl D.S. of 0.8-1.0 and a molecular weight ranging from three million to sixty million.

TABLE

| Extraction Fluid pH | Extraction Period | Total Extraction Time | Range in percent of Medicament Extracted (Accumulative) |
|---------------------|-------------------|-----------------------|---------------------------------------------------------|
| 60                  |                   |                       |                                                         |
| 1.5.....            | 5 min.....        | 5 min.....            | 6-12                                                    |
| 1.5.....            | 55 min.....       | 1 hr.....             | 20-30                                                   |
| 7.5.....            | 1 hr.....         | 2 hr.....             | 30-45                                                   |
| 7.5.....            | 2 hr.....         | 4 hr.....             | 40-55                                                   |
| 7.5.....            | 4 hr.....         | 8 hr.....             | 50-75                                                   |
| 7.5.....            | 8 hr.....         | 16 hr.....            | 80-100                                                  |

The following examples illustrate the preparation of additional delayed release compositions.

#### Example I

Small amounts of methanol were mixed into benzyl dextran having a benzyl D.S. of 0.8-1.0 (18.0 g., -40 mesh) until a soft plastic mass was obtained (approximately 20 ml. methanol required). Amphetamine sul-

phate (2.0 g.) was dissolved in water (2 ml.) and the solution was mixed into the plastic mass. The resulting mixture of benzyl dextran-amphetamine sulphate was then dried at 60° C. under vacuum and the dried cake was crushed to -20 to +40 mesh granules for testing. The results are shown in Table II below.

*Example II*

This composition was prepared exactly as described in Example I except that half the amount of amphetamine sulphate was used and the latter was dissolved directly in the methanol suspension (no water used). The results are shown in Table II below.

*Example III*

This composition was prepared as described in Example I except that less methanol was used (5 ml. total) and a ratio of 8.5 parts of benzyl dextran to 1.5 parts of amphetamine sulphate was used. The results are shown in Table II below.

*Example IV*

Dextroamphetamine (0.53 g.) was added to methanol (10 ml.) and the solution was mixed into benzyl dextran of the character used in Example I (10.0 g., -40 mesh), adding it in small amounts. The resulting soft mass was dried at 60° C. under vacuum and the dried cake was crushed to -20 to +40 mesh granules. The results are shown in Table II below.

*Example V*

Small amounts of dioxalane were mixed into benzyl dextran of the type used in Example I (10.0 g., -40 mesh) until a total of 10 ml. was added. The past was heated to 90° C. and the amphetamine sulphate (1.3 g.) was added. The soft mass was dried at 60° C. under vacuum, and the dry cake was crushed to -10 to +20 mesh granules.

The extraction data obtained from Examples I-V are given in Table II below.

TABLE II

| Example | Size of Granules, Mesh | Amphetamine Percent | Amphetamine Extract Simulated Gastric Fluid Percent |          | Amphet. Extr. Sim. Intest. Fluid Percent |        |
|---------|------------------------|---------------------|-----------------------------------------------------|----------|------------------------------------------|--------|
|         |                        |                     | 1 Hr.                                               | 1.5 Hrs. | 1 Hr.                                    | 2 Hrs. |
| 1       | -20 +40                | 7.7                 | 45.8                                                |          | 15.2                                     | 13.0   |
| 2       | -20 +40                | 4.0                 | 52.9                                                |          | 22.0                                     | 11.2   |
| 3       | -20 +40                | 9.9                 | 51.1                                                |          | 18.4                                     | 17.4   |
| 4       | -20 +40                | 4.5                 | 29.0                                                |          | 16.7                                     | 12.5   |
| 5       | -10 +20                | 8.1                 |                                                     | 43.5     | 17.3                                     | 11.4   |

*Example VI*

In this example a delayed release medicament was prepared with chlorprophenyridamine following the procedure described in Example I, using a benzyl dextran having a molecular weight ranging from three million to sixty million, and a benzyl D.S. ranging from 0.8 to 1.0. The final dried cake was crushed to -20 to +40 mesh granules. Administered in capsule form, it gave a satisfactory rate of release of the medicament over a period of 8 to 12 hours.

*Example VII*

In this example a delayed release medicament was prepared as described in Example VI using promethazine with similar results.

*Example VIII*

In this experiment a dextroamphetamine sulphate-benzyl dextran delayed release medicament prepared as described in Example I was used. To achieve a dosage of 10 mg. of d-amphetamine sulphate (a desirable dosage figure in the light of present knowledge) 66.7 mg. of the d-amphetamine benzyl dextran was found to be necessary. This amount of material was mixed with a suitable excipient for filling into hard gelatine capsules. A suitable formulation is as follows:

|                              | Gm.    |
|------------------------------|--------|
| d-Amphetamine-benzyl dextran | 0.0667 |
| Starch #10 granules          | 0.1653 |
| Magnesium stearate           | 0.0080 |
|                              | <hr/>  |
| Total fill                   | 0.2400 |

The amount of the excipient can be varied as desired for different size capsules. The delayed release properties were determined as follows:

One capsule, each containing 0.0667 gm. d-amphetamine sulphate-benzyl dextran, was ingested by each of two patients in the morning before breakfast. Urinary collections were made representing 2, 4, 8, 16, 24, 48 and 72 hours following administration of the drug. The urine samples were analyzed for their amphetamine content. The results obtained are shown in the following table.

TABLE

[Amphetamine sulphate content of urine (mgs.)]

|                                                   | Patient A   |       |                                                  | Patient B   |       |         |
|---------------------------------------------------|-------------|-------|--------------------------------------------------|-------------|-------|---------|
|                                                   | Time, Hours | Total | Per Hr.                                          | Time, Hours | Total | Per Hr. |
| 2                                                 |             | 302   | 151                                              | 2           |       | 62      |
| 4                                                 |             | 765   | 382                                              | 4           |       | 692     |
| 8                                                 |             | 1,330 | 332                                              | 8           |       | 392     |
| 16                                                |             | 2,227 | 278                                              | 16          |       | 2,670   |
| 24                                                |             | 3,107 | 389                                              | 24          |       | 1,622   |
| 48                                                |             | 1,475 | 61                                               | 48          |       | 1,491   |
| 72                                                |             | 195   | 8                                                | 72          |       | 498     |
| Total recovered, 9,140 mg. Percent recovered, 94. |             |       | Total recovered, 7,83 mg. Percent recovered, 78. |             |       |         |

If preferred, the benzyl dextran-medicament particles can be incorporated in tablet form, according to the practice of the trade, using inert excipients.

Now having described the invention, what is claimed is:

1. In a method of producing a therapeutic composition for oral ingestion to provide a gradual release of medicament over an extended period of time in the intestinal tract and comprising preparing a fluid paste of benzyl dextran and methanol and incorporating into the benzyl dextran paste a medicament and drying the resulting mixture, the improvement consisting of employing a benzyl dextran having a molecular weight between 3,000,000 and 60,000,000 and having a D.S. of benzyl ranging between 0.8 and 1.0, and wherein the particle size of the dried product is on the order of -20 to +40 mesh and which product contains up to 5% benzyl alcohol.

2. A pharmaceutical product produced in accordance with the process of claim 1.

References Cited in the file of this patent

UNITED STATES PATENTS

- |           |               |               |
|-----------|---------------|---------------|
| 2,989,518 | Novak         | June 20, 1961 |
| 3,063,905 | Novak         | Nov. 13, 1962 |
| 3,063,906 | Heckel et al. | Nov. 13, 1962 |